

A. R. & N. B. Reynolds,

Tempering Steel.

No. 70471.

Patented Nov. 5, 1857.

Fig. 1.



Fig. 2.



Witnesses.

Jed D. Patten, A. R. Reynolds & N. B. Reynolds,  
Thos. F. Chamberlain, By attorney A. B. Stoughton,

Inventors.

# United States Patent Office.

ASA R. REYNOLDS AND NAPOLEON B. REYNOLDS, OF AUBURN, NEW YORK,

Letters Patent No. 70,471, dated November 5, 1867.

## IMPROVEMENT IN TEMPERING STEEL.

The Schedule referred to in these Letters Patent and making part of the same.

TO ALL WHOM IT MAY CONCERN:

Be it known that we, ASA R. REYNOLDS and NAPOLEON B. REYNOLDS, of Auburn, in the county of Cayuga, and State of New York, have invented certain new and useful Improvements in Tempering Cutlery, or cutting instruments, made in whole or in part of steel, under a head of flowing water; and we do hereby declare the following to be a full, clear, and exact description of the same, reference being had to the accompanying drawings, making a part of this specification, in which—

Figure 1 represents a top plan of a guide or apparatus by which the tempering under a head of flowing water may be readily and uniformly done.

Figure 2 represents a vertical section through the guide or apparatus.

Similar letters of reference, where they occur in the separate figures, denote like parts in both of the drawings.

Our invention relates to the tempering of articles made in whole or in part of steel, under a head of flowing water, by which means great uniformity and fineness of granulation of the metal is attained, and without so high a heat as is usual in tempering cutlery or cutting instruments, and without its liability to crack or warp.

To enable others skilled in the art to make and use our invention, we will proceed to describe the same with reference to the drawings.

A represents a horizontal chamber, of a pyramidal form, and enclosed by suitably strong metallic sides, B, and end piece, C. Into the small end of this horizontal pyramidal chamber a water pipe, D, is introduced, which may extend upwards to a tank or reservoir, or which may connect otherwise with a head of water of sufficient height for the purpose. Through the base or end of this chamber there is an opening, E, of such form as may best suit the shape or size of the article to be tempered, or so as to best throw the current of water upon the special parts of the article to be tempered. In front of the end or base-plate C there is a guide-roller, F, between which and the projecting flanges G the article, such as a plane-iron, chisel, sickle-section, or other similar thing of an uniform thickness, and of parallel or nearly parallel sides, is inserted, and which rests upon the shelf a, and is thus supported in proper position with regard to the flow of water against it through the opening E, as to remain firmly in place against the force of the current, and be easily and readily inserted and removed therefrom. Around and underneath the article so placed there is sufficient free and unincumbered space or water-way for the flow of water to freely escape the moment after striking against the article that is being tempered.

For ordinary tempering, the head of water may be, or equal to a pressure of, seven or eight feet in height, but may vary according to the temperature or heat taken in the article to be tempered. We find, in practice, that the higher the head, or the greater the pressure of water in or through the guide, or tempering-head, or nozzle, the less the steel need be heated; and that the less the heat in the steel, the better is the temper, as the granulation of the metal is proportionately finer. When the flow of water is rapid and strong, it quickly absorbs or takes up the heat from the steel, and as suddenly carries it away, to be succeeded by a continuous sudden subjection and passing off, and thus instantaneously tempers or granulates the particles of steel.

For tempering axes, hatchets, files, or other similar articles, where there is a greater quantity of steel, and the sides not parallel, we propose to use two or more of these guides or tempering-heads, placed opposite to each other, and the axe, hatchet, file, or other article, placed between the two heads, so that there shall be a flow or current of water upon each side, and an escape for the water all around except at the points of support.

It is important that the article should be quickly placed in the position where the water is to strike it, because the proper heat is to be preserved, and it runs out quickly after being raised from the bath of molten metal, in which we prefer to heat it, as a more uniform degree of heat is thus attained.

The column of flowing water may strike nearly central of the article to be tempered, which insures that part of it to be properly tempered, which is not the case when it is dipped into water end or edgewise; and by our mode the temper runs from the centre to the edges, whilst, by the dipping or immersion in water at rest, it runs from the edges to the centre, and is so very hard at the edges as to be with difficulty ground off, whilst the metal, when thin, will fly like glass when strained, and is soft in the centre. By our plan the centre is first tempered, and the temper runs to the edges, leaving all portions of a uniform degree of hardness, and of most perfect granulation of metal.

Having thus fully described our invention, what we claim is—

Tempering articles made in whole or in part of steel, by means of a head of flowing water, and a guiding and holding, hardening, or tempering-head, substantially as herein described.

ASA R. REYNOLDS,  
NAPOLEON B. REYNOLDS.

Witnesses:

C. MACDONAGLASS,  
E. L. PARSONS.